

## UNITED STATES PATENT OFFICE

2,527,279

## ANTIOXIDANTS FOR MINERAL OIL LUBRICANTS AND COMPOSITIONS CONTAINING THE SAME

Herschel G. Smith, Wallingford, and Troy L. Cantrell, Lansdowne, Pa., and John G. Peters, Audubon, N. J., assignors to Gulf Oil Corporation, Pittsburgh, Pa., a corporation of Pennsylvania

No Drawing. Application November 17, 1949,  
Serial No. 127,992

18 Claims. (Cl. 252—47.5)

**1**  
This invention relates to antioxidants for mineral oil lubricants and compositions containing the same, and more particularly, it relates to addition agents for mineral oil lubricants which inhibit the oxidative deterioration of said lubricants.

In the lubrication of internal combustion engines of all types, particularly when severe operating conditions are encountered, plain mineral lubricating oils often prove unsatisfactory in service because of the oxidative deterioration of the oil, with the attendant deposition on the engine surfaces of varnish, gum or sludge. Furthermore, many lubricating oil compositions which may be highly satisfactory for the lubrication of other mechanisms have been found wholly unsuitable for use as turbine oils.

The formation of varnishes, gums and sludges on engine surfaces is due at least in part to oxidation effects on mineral lubricating oils. In turbine oils the problem of oxidation is further aggravated, because in normal use turbine oils rapidly become contaminated with water.

It is an object of this invention, therefore, to provide an addition agent for mineral oil lubricants which will inhibit the oxidative deterioration of such lubricants.

It is a further object of this invention to provide improved mineral oil lubricant compositions which are remarkably stable against oxidation under service conditions.

These and other objects are accomplished by the present invention wherein an addition agent for mineral oil lubricants is prepared by condensing a di (alkylphenol) sulfide, N-dimethylaniline and formaldehyde in the presence of an activated clay as a catalyst, and recovering the condensation product. The condensation product so obtained is a liquid product which, when added to mineral oil lubricants, confers an excellent stability against deterioration by oxidation. In addition, bearing corrosion inhibiting properties are conferred on the oil. Such condensation products and the mineral oil lubricant compositions containing them are believed to be novel and are considered parts of our invention. Contrary to what may be expected from the nature of the reactants, we do not obtain highly condensed, insoluble resinous products. On the contrary, when the above reactants are condensed

**2**  
in accordance with our invention, there are obtained liquid condensation products which are non-resinous and which are readily soluble in mineral oils.

5 In performing the condensation, the reactants are mixed and heated to a maximum temperature of 350° F. We have found that if the temperature of 350° F. is exceeded to any substantial extent, the condensation product formed tends to 10 be resinous and insoluble. In general, the preferred temperature for the condensation ranges from 150° to 300° F.

The proportions of the reactants vary as follows. The di (alkylphenol) sulfide is employed in 15 an amount of 1 mol, N-dimethylaniline in an amount of from 1 to 2 mols, and formaldehyde in an amount of from 1 to 2 mols. Ordinarily, it is preferred to use from 5 to 10 per cent by weight of the activated clay catalyst, based on the total 20 weight of the reactants. However, smaller amounts, as low as 1 per cent by weight, and larger amounts, as high as 20 per cent by weight, may also be employed; but larger amounts than about 10 per cent by weight are ordinarily not necessary.

The di (alkylphenol) sulfides used in preparing our new compounds have the formula



35 where R is an alkyl group of from 4 to 12 carbon atoms and x is the integer 1 or 2. As is known in the art, these compounds are readily prepared by reacting an alkyl phenol with sulfur monochloride or sulfur dichloride, as the case may be.

40 The alkyl phenols employed are mono-alkyl phenols having from 4 to 12 carbon atoms, that is, the alkyl substituent is butyl, t-butyl, amyl, sec-amyl, t-amyl, hexyl, heptyl, octyl, iso-octyl (tetramethylbutyl), decyl, triisobutyl or the like.

45 The preferred alkyl phenols are prepared by alkylating phenol with suitable olefins in the presence of concentrated sulfuric acid as a catalyst. A preferred alkyl phenol is p-tetramethylbutyl phenol obtained by alkylating phenol with diisobutylene, and the mono- and di-(iso-

octylphenol) sulfides obtained therefrom are preferred di (alkylphenol) sulfides for the purposes of this invention.

In lieu of formaldehyde, any formaldehyde-yielding compound, such as paraformaldehyde, dioxymethylene and trioxymethylene may be employed in the condensation. In such case, the amount of formaldehyde-yielding compound used is based on the equivalent number of mols of formaldehyde yielded within the range of proportions of formaldehyde set forth hereinabove. Accordingly, as used in the appended claims, the term "formaldehyde" is intended to include formaldehyde-yielding compounds as well as formaldehyde itself.

Various activated clays are employed as catalysts in accordance with our invention. Such materials are well known in the art and comprise a natural clay, such as bentonite, fuller's earth, montmorillonite, floridin and smectite, which has been acid treated in order to activate the clay. Such materials are described in U. S. Patent 1,898,165, for example. A preferred activated clay is activated montmorillonite sold under the name of Filtrol.

In preparing our new addition agents, the reactants and catalysts are placed into a reaction vessel which is then closed and the mixture heated with agitation under reflux until all of the formaldehyde or formaldehyde-yielding compound has been consumed. At this time, the water which is formed as a result of the condensation is removed, preferably under vacuum, and the dehydrated condensation product is then filtered to remove the activated clay catalyst. In some instances, it is desirable to prepare our new addition agent in a concentrate in a mineral lubricating oil which may then be diluted with additional oil to the concentration desired in the final lubricating composition. In such instances, the mineral lubricating oil may be added in a suitable amount, say in a weight equal to the weight of reactants, to the reaction mixture in the reaction vessel, and the condensation product obtained will then be a concentrated solution of the addition agent in the mineral lubricating oil.

The condensation products obtained in accordance with our invention are non-resinous liquids. While the exact nature of the chemical composition of the condensation products is unknown, all of the three reactants enter into a final unitary product. The exact manner in which the catalyst influences the reaction is unknown. However, regardless of any theory involved, the use of an activated clay catalyst is an essential feature of our invention, since if the catalyst is omitted, black, insoluble, resinous condensation products are obtained.

The following examples illustrate the preparation of our new addition agent. Unless otherwise indicated, all parts are by weight.

*Example I.*—Into a stainless steel reaction vessel, there were charged 442 parts of di (iso-octylphenol) sulfide, 242 parts of N-dimethylaniline, 68 parts of activated montmorillonite (Filtrol) and 170 parts of a 37 per cent by weight aqueous solution of formaldehyde. The reactants were in the molar proportions of 1 mol of the di (iso-octylphenol) sulfide, 2 mols of the N-dimethylaniline and 2 mols of the formaldehyde. The mixture was heated with agitation and refluxed for a period of 5 hours. Thereafter, the temperature was raised to 280° F. and all water, both that added with the formaldehyde and formed in the reaction, was distilled off. The

dried product was filtered and had the following properties:

|                   |     |
|-------------------|-----|
| Gravity, °API     | 6.7 |
| Sulfur, per cent  | 4.0 |
| Neutralization No | 3.1 |

*Example II.*—Three hundred fifty-eight (358) parts of di-(t-amylphenol) sulfide, 242 parts of N-dimethylaniline, 68 parts of activated montmorillonite (Filtrol) and 170 parts of a 37 per cent by weight aqueous solution of formaldehyde were placed into a stainless steel reaction vessel. The reactants were in the molar proportions of 1 mol of the di (t-amylphenol) sulfide, 2 mols of the N-dimethylaniline and 2 mols of the formaldehyde. The vessel was then closed and the mixture heated with agitation and refluxed for 5 hours. The temperature was then raised to 280° F. to distill off all water, thereby dehydrating the liquid product. The product was then filtered and had the following properties:

|                   |     |
|-------------------|-----|
| Gravity, °API     | 5.1 |
| Sulfur, per cent  | 5.7 |
| Neutralization No | 3.4 |

*Example III.*—Into a stainless steel reaction vessel, there were charged 442 parts of di (iso-octylphenol) sulfide, 121 parts of N-dimethylaniline, 34 parts of activated montmorillonite (Filtrol) and 170 parts of a 37 per cent by weight aqueous solution of formaldehyde. The reactants were in the molar proportions of 1 mol of the di (iso-octylphenol) sulfide, 1 mol of the N-dimethylaniline and 2 mols of the formaldehyde. The reactants were reacted under the conditions shown in Example I. The liquid reaction product had the following properties:

|                   |     |
|-------------------|-----|
| Gravity, °API     | 5.9 |
| Sulfur, per cent  | 9.8 |
| Neutralization No | 4.9 |

The condensation products obtained in accordance with the above disclosure from di (alkylphenol) sulfides, N-dimethylaniline and formaldehyde in the presence of an activated clay catalyst are excellent addition agents for mineral oil lubricants. They are readily soluble in all types of mineral oils, that is paraffinic, naphthenic or mixed base mineral oils and can be blended with mineral oils in high proportions to form concentrated solutions thereof, which may then be diluted down to the proportions desired in the final mineral oil lubricant composition. As stated, our new addition agents are remarkably effective in inhibiting the oxidative deterioration of mineral oil lubricant compositions. For this purpose, small amounts of our new addition agents are generally sufficient. For example, our addition agents may be added to mineral lubricating oils in minor amounts, say from 0.1 to 10 per cent by weight on the mineral oil, sufficient to inhibit the oxidative deterioration of the oil. Larger amounts of our new addition agents may be used if desired but it is ordinarily unnecessary to do so. In addition, to inhibiting oxidative deterioration, our new addition agents are also effective bearing corrosion inhibitors.

The following examples illustrate the advantageous effects of our new addition agents. In the following examples, the base oil and the same oil blended with our new addition agents are subjected to a standard oxidation test which measures the stability of the oils to oxidation. The oxidation test referred to is a standard test designated ASTM D943-47T. Briefly, the test

comprises subjecting the oil sample to oxygen at a temperature of 95° C. (203° F.) in the presence of water and an iron-copper catalyst, and determining the time required to build up a neutralization number of 2. The flow of oxygen is maintained at 3 liters per hour. The effective stability to oxidation of mineral oil lubricant compositions containing our new addition agents is illustrated by the results shown in the following examples.

**Example IV.**—A turbine lubricating oil was blended with 0.5 per cent by volume of the additive prepared according to Example I. A comparison of the base oil and improved oil showed the following:

|                                                                        | Base Oil | Improved Oil |
|------------------------------------------------------------------------|----------|--------------|
| Gravity, °API                                                          | 29.4     | 29.4         |
| Viscosity, S.U.V.:                                                     |          |              |
| 70° F.                                                                 | 785      | 781          |
| 100° F.                                                                | 305      | 304          |
| 210° F.                                                                | 53.0     | 52.9         |
| Viscosity Index                                                        |          |              |
| Flash, OC: °F                                                          | 100      | 100          |
| Fire, OC: °F                                                           | 450      | 450          |
| Color, N.P.A.                                                          | 510      | 510          |
| Oxidation Test, ASTM D943-47T: Time Oxidized, Hr. for Neut. No. of 2.0 | 2.0      | 2.0          |
|                                                                        | 100      | 2,100        |

**Example V.**—A turbine lubricating oil was blended with 0.5 per cent by volume of the compound of Example II. The blended and unblended oil had the following properties:

|                                                                        | Base Oil | Improved Oil |
|------------------------------------------------------------------------|----------|--------------|
| Gravity, °API                                                          | 25.2     | 29.2         |
| Color, N.P.A.                                                          | 2.75     | 3.0          |
| Neutralization No.                                                     | 0.02     | 0.03         |
| Oxidation Test, ASTM D943-47T: Time Oxidized, Hr. for Neut. No. of 2.0 | 90       | 1,600        |

The above examples show the notable oxidation stability imparted to mineral oil lubricant compositions by the use of our new addition agents. Mineral oil lubricant compositions containing our new addition agents are therefore eminently suited for use where the operating conditions are extremely severe, as in Diesel, tank and truck engines, and in the lubrication of steam turbines.

The effects of our new addition agents cannot be readily accounted for and cannot be predicted from the nature of the reactants. Thus, condensation products prepared from other functionally similar compounds have been found to be either pro-oxidant or to show no antioxidant effects whatsoever. For example, we have prepared condensation products similar to our new addition agents by substituting aniline for the dimethylaniline. The resulting condensation products were found to be entirely unsuitable for inhibiting the oxidative deterioration of mineral oil lubricant compositions.

While we have shown in the examples the preparation of compounded lubricating oils, our invention is not limited thereto but comprises all mineral oil lubricant compositions containing our new addition agents, such as greases and the like. If desired, other known addition agents may be incorporated into the lubricant compositions prepared in accordance with our invention. For example, pour point depressants, extreme-pressure agents, viscosity index improvers and the like may be added.

Resort may be had to such modifications and

variations as fall within the spirit of the invention and the scope of the appended claims.

We claim:

1. The process of preparing an addition agent for mineral oil lubricants which comprises heating 1 mol of a di (alkylphenol) sulfide having the formula

10



15 wherein R is an alkyl group of from 4 to 12 carbon atoms and x is an integer from 1 to 2, 1 to 2 mols of N-dimethylaniline, and 1 to 2 mols of formaldehyde in the presence of an activated clay catalyst at a temperature not in excess of

350° F. to condense together the three reactants, and recovering the condensation product.

2. The process of preparing an addition agent for mineral oil lubricants which comprises heating 1 mol of a di (alkylphenol) sulfide having the formula

20  
30



wherein R is an alkyl group of from 4 to 12 carbon atoms and x is an integer from 1 to 2, 1 to 2 mols of N-dimethylaniline, and 1 to 2 mols of formaldehyde in the presence of an activated clay catalyst at a temperature of from 150° to 300° F. to condense together the three reactants, and recovering the condensation product.

3. The process of claim 1, wherein x is 2 and R is the iso-octyl radical.

4. The process of preparing an addition agent for mineral oil lubricants which comprises adding 1 mol of a di (alkylphenol) sulfide having the formula

40  
50



wherein R is an alkyl group of from 4 to 12 carbon atoms and x is an integer from 1 to 2, 1 to 2 mols of N-dimethylaniline, 1 to 2 mols of formaldehyde and from 5 to 10 per cent by weight on the foregoing reactants of an activated clay catalyst to a mineral lubricating oil, heating the mixture at a temperature of from 150° to 300° F. to condense together the three reactants, and recovering a solution of the condensation product in the mineral lubricating oil.

5. The process of preparing an addition agent for mineral oil lubricants which comprises heating 1 mol of di (iso-octylphenol) sulfide, 2 mols of N-dimethylaniline and 2 mols of formaldehyde in the presence of an activated clay catalyst at a temperature of from 150° to 300° F. to condense together the three reactants, and recovering the condensation product.

6. The process of preparing an addition agent for mineral oil lubricants which comprises heating 1 mol of di (t-amylphenol) sulfide, 2 mols of N-dimethylaniline and 2 mols of formaldehyde in the presence of an activated clay cata-

70  
75

lyst at a temperature of from 150° to 300° F. to condense together the three reactants, and recovering the condensation product.

7. The process of preparing an addition agent for mineral oil lubricants which comprises heating 1 mol of di (iso-octylphenol) sulfide, 1 mol of N-dimethylaniline and 2 mols of formaldehyde in the presence of an activated clay catalyst at a temperature of from 150° to 300° F. to condense together the three reactants, and recovering the condensation product.

8. A non-resinous condensation product of 1 mol of a di (alkylphenol) sulfide having the formula



wherein R is an alkyl group of from 4 to 12 carbon atoms and x is an integer from 1 to 2, 1 to 2 mols of N-dimethylaniline and 1 to 2 mols of formaldehyde, said product being obtained by the process of claim 1.

9. The product of claim 8, wherein x is 2 and R is the iso-octyl radical.

10. A non-resinous condensation product of 1 mol of di (iso-octylphenol) sulfide, 2 mols of N-dimethylaniline and 2 mols of formaldehyde, said product being obtained by the process of claim 5.

11. A non-resinous condensation product of 1 mol of di (t-amylphenol) sulfide, 2 mols of N-dimethylaniline and 2 mols of formaldehyde, said product being obtained by the process of claim 6.

12. A non-resinous condensation product of 1 mol of di (iso-octylphenol) sulfide, 1 mol of N-dimethylaniline and 2 mols of formaldehyde, said product being obtained by the process of claim 7.

13. A lubricant composition comprising a major amount of a mineral lubricating oil, and a minor amount, sufficient to inhibit the oxidative deterioration of said oil, of a non-resinous condensation product of 1 mol of a di (alkylphenol) sulfide having the formula



wherein R is an alkyl group of from 4 to 12 carbon atoms and x is an integer from 1 to 2, 1 to 2 mols of N-dimethylaniline and 1 to 2 mols of formaldehyde, said product being obtained by the process of claim 1.

14. The composition of claim 13, wherein x is 2 and R is the iso-octyl radical.

15. A lubricant composition comprising a major amount of a mineral lubricating oil, and a minor amount, from 0.1 to 10 per cent by weight of said oil, of a non-resinous condensation product of 1 mol of a di (alkylphenol) sulfide having the formula



wherein R is an alkyl group of from 4 to 12 carbon atoms and x is an integer from 1 to 2, 1 to 2 mols of N-dimethylaniline and 1 to 2 mols of formaldehyde, said product being obtained by the process of claim 1.

16. A lubricant composition comprising a major amount of a mineral lubricating oil, and a minor amount, sufficient to inhibit the oxidative deterioration of said oil, of a non-resinous condensation product of 1 mol of di (iso-octylphenol) sulfide, 2 mols of N-dimethylaniline and 2 mols of formaldehyde, said product being obtained by the process of claim 5.

17. A lubricant composition comprising a major amount of a mineral lubricating oil and a minor amount, sufficient to inhibit the oxidative deterioration of said oil, of a non-resinous condensation product of 1 mol of di (t-amylphenol) sulfide, 2 mols of N-dimethylaniline and 2 mols of formaldehyde, said product being obtained by the process of claim 6.

18. A lubricant composition comprising a major amount of a mineral lubricating oil, and a minor amount, sufficient to inhibit the oxidative deterioration of said oil, of a non-resinous condensation product of 1 mol of di (iso-octylphenol) sulfide, 1 mol of N-dimethylaniline and 2 mols of formaldehyde, said product being obtained by the process of claim 7.

HERSCHEL G. SMITH.  
TROY L. CANTRELL.  
JOHN G. PETERS.

No references cited.